

Nov. 19, 1968

H. W. H. JONES, ET AL.

**3,411,720**

## PRODUCTION OF MECHANICAL PULP FROM WOOD CHIPS

Filed Aug. 18, 1966

2 Sheets-Sheet 1



INVENTOR  
Howard W. H. Jones  
Donald E. Hellmer  
BY Wm. Marshall,  
MacKee & Hamby,  
PATENT AGENT

Nov. 19, 1968

H. W. H. JONES ET AL

**3,411,720**

## PRODUCTION OF MECHANICAL PULP FROM WOOD CHIPS

Filed Aug. 18, 1966

2 Sheets-Sheet 2



Fig. 3.

Fig. 56.



Fig. 5a.



Fig. 4.

Fig. 4.

INVENTOR  
Howard W. Jones  
Donald E. Killeen  
BY Weir, Marshall,  
Mackay & Hamby  
PATENT AGENT

BY Weir, Marshall,  
MacRae & Hamby  
PATENT AGENT

1

3,411,720

## PRODUCTION OF MECHANICAL PULP FROM WOOD CHIPS

Howard W. H. Jones and Donald E. Helleur, Grand'Mere, Quebec, Canada, assignors to Consolidated Paper (Bahamas) Limited, Nassau, Bahamas  
Continuation-in-part of application Ser. No. 170,110, Jan. 31, 1962. This application Aug. 18, 1966, Ser. No. 573,271  
6 Claims. (Cl. 241—28)

### ABSTRACT OF THE DISCLOSURE

A mechanical process for treating raw, uncooked wood chips in which increased amounts of energy are expended on the wood material to increase the strength of the resulting pulp. Raw wood chips are fed centrally into a treatment area between a stationary disc and a rotating disc and are caused to move radially outwards over a sinuous path. The discharge at the periphery is restricted to increase the energy expended on the wood material, and the treatment area is enclosed to permit the steam generated to increase the pressure in the area.

This application is a continuation-in-part of application Ser. No. 170,110 filed Jan. 31, 1962, and now abandoned.

This invention relates to a process for converting raw wood by mechanical means into a wood pulp, and in particular, it relates to a mechanical pulping process for converting raw uncooked chips into a wood pulp.

Wood pulps which are produced by a process employing mechanical means only, that is which do not rely on the addition of chemicals in the process, are known as mechanical pulps. Water or substances occurring naturally in the wood may be used in a process for producing a mechanical pulp, but the addition of chemicals does not take place for the pulp in its unbleached form; however, for bleached grades of mechanical pulp, chemicals are added which do not essentially change the yield of the unbleached pulp, but which do make the pulp appear brighter and whiter. On the other hand, when chemicals are added to convert raw wood into a pulp, the resulting pulp is known as a chemical pulp. If a process for producing a pulp uses a combination of a mechanical means and a chemical means, the resulting pulp is referred to as a high yield pulp or a semi-chemical pulp or a mechano-chemical pulp. For all these pulps the yield is less than for a pure mechanical pulp, the lowest yield is for the purely chemical pulp and the yield for the mechano-chemical pulp is close to the mechanical pulp yield. This invention pertains to a mechanical pulping process which converts raw wood in the form of chips into a mechanical wood pulp.

A known process for making a mechanical wood pulp forces whole logs against a large revolving grindstone. The pulp produced by this process is commonly referred to as groundwood. In general, groundwood is cheaper than other known types of wood pulp, and the process provides more pulp for a given weight of wood than other pulping processes. The groundwood pulps, however, do not always have the necessary properties to give a finished paper product of the required quality. For example, the groundwood pulp, or paper made from groundwood pulp, may not have satisfactory runnability on a paper machine or in a printing press, or other properties in the finished paper product may not be satisfactory. As a result, various percentages of chemical and/or semi-chemical pulps are incorporated with the groundwood pulp to give the mixed-furnish or the finished product the required properties.

2

Since chemical pulps are expensive, every effort is made to keep the percentage of the chemical pulp content as low as possible. It will be apparent that any improvement in the properties of a mechanical pulp which reduces the chemical pulp content necessary for a given quality of paper, would be very desirable.

In the past, refinements in the groundwood process have been made which improve the properties of the groundwood pulp, and this has resulted in a reduction of the chemical pulp content required for a given quality in the finished product. Intensive studies have been made of the operating variables in the groundwood process, and the ranges of groundwood pulp properties that may be achieved by the controlled variation of these variables are known. It has been found, very generally, that the more energy used or consumed in the grinding process, the stronger will be the resulting pulp. There are, however, limits to the increase in strength that can be obtained by increasing the energy used per ton of pulp processed. One limitation is that the drainage rate decreases fairly quickly as more energy per ton is used in the groundwood process. The energy input cannot be increased past a point where the drainage rate or "freeness" becomes too low for a paper machine to operate properly. Thus, in the conventional groundwood process there is a definite limitation to the strength that can be achieved.

In another form of groundwood process it is known to subject whole logs to a coarse grinding step, to screen the resulting wood material, to refine the screen rejected material in a disc mill, and to combine the ground pulp with the pulp from the disc mill. This provides a pulp with strength properties generally less than or of the same order as that of conventional groundwood pulp. With this process also there are limitations to the power than can be applied to or absorbed by the pulp and consequently there are limitations to the resulting strength.

Recently attempts have been made to refine mill chips, shavings, etc. in a disc mill or disc refiner to produce a mechanical pulp similar to conventional groundwood pulp. Because the wood material in this process is subjected to a tearing and shearing action closely akin to grinding, the characteristics of the pulp produced are very similar to the characteristics of groundwood pulp. Consequently the process is said to produce "groundwood from chips." The strength of the pulp produced by the groundwood from chips process is generally less than or of the same order as that of conventional groundwood pulp.

The present invention seeks to provide a process for making an improved mechanical pulp from conventional wood chips. With the process of this invention increased amounts of energy can be absorbed by the wood material with a resulting increase in strength. The characteristics or properties of the pulp produced are quite distinguishable from the aforementioned conventional groundwood pulp or from groundwood pulp from chips.

It is therefore an object of this invention to provide an improved process for making a mechanical pulp from wood chips.

It is another object of this invention to provide a process for producing a mechanical pulp that has a greater strength than comparable prior art mechanical pulps.

Further objects and advantages of the invention will be apparent from the following description taken in conjunction with the accompanying drawings in which,

FIGURE 1 is a flow sheet in block form of an overall mechanical pulp process in accordance with one embodiment of the invention.

FIGURE 2 is a simplified side view partly in section, of part of a disc refiner that may be used in the process of the invention,

FIGURE 3 is a fragmentary plan view of the plates used in the disc refiner of FIGURE 2.

FIGURE 4 is a side view, partly in section, of separating apparatus that may be used in the process of the invention, and

FIGURES 5a and 5b are graphs showing examples of results obtained using the process of the invention.

Briefly, the process of the invention in a basic form is for the treatment of wood chips comprising the steps of feeding wood chips to a central area, moving the wood chips from said central area radially along a sinuous path, during movement of said chips along said path subjecting said chips to a continuously recurring flexing action to fiberize said chips, restricting the movement of said chips along said path to prolong the period of treatment, generating steam with the heat created by the flexing action and maintaining the steam at a desired pressure.

Referring now to FIGURE 1, which shows a flow diagram in block form of the pulping process in accordance with one embodiment of the invention, the designation number 10 represents a chip bin containing raw uncooked wood chips. Wood chips from chip bin 10 are conveyed to a refiner stage 11 comprising a disc refiner which will be described in more detail hereinafter. The wood chips in refiner stage 11 are subjected to a continuously recurring flexing action to fiberize the chips. The movement of the wood material through the refiner in stage 11 is restricted to prolong the treatment and permit a required amount of energy to be expended on the material. The output from refiner stage 11 is screened in coarse screens 12 with the rejected material being returned to refiner stage 11 for further treatment and the accepted material being passed to fine screens 14. The rejected wood material from fine screens 14 is fed into a mixing tank 15 and the accepted material is passed to a centrifugal separator or cleaner stage 16. The separator stage 16 may comprise a centrifugal separator of the vortex pressure drop type to be described in more detail in connection with FIGURE 4. This type of cleaner or separator is known in the prior art for separating small amounts of undesirable wood material and dirt from a wood material being processed. The acceptable pulp from separator stage 16 may be fed to a thickening stage 17 or similar final stage, and the non-acceptable wood material is transferred to mixing tank 15.

It is important that the acceptable pulp be removed after the first stage of refining so that it will not be over-processed in subsequent refining stages. This separation of the pulp after the first stage permits the necessary amount of processing to be used in the first stage to get a maximum yield of a good strength pulp from the first stage, and it also permits a suitable amount of additional refining to be given to those fractions of wood material which require it.

From the mixing tank 15 the wood material is transferred to a centrifugal separator 20 where it is separated into two fractions which may be referred to as a coarse fraction and a less coarse fraction. The separator 20 is similar to that used in separator stage 16, except that it is operated differently in order to classify the material into two major fractions. As will be described subsequently, the stage 20 separator is operated at hydraulic pressures lower and reject rates higher than those in the more conventional separator stages 16, 26 and 27. Each of these two fractions from stage 20 are then subjected to a second stage of refining. The coarse fraction goes through a drainage stage 21 to a refiner stage 22. The block representing refiner stage 22 is labelled "Refiners, Stage 2-C" meaning that it is a refiner refining a second stage of wood material and the wood material is the coarse fraction. The refiner stage 22 may comprise a disc refiner conventional in all respects and used in a conventional manner.

The less coarse fraction goes through drainage stage 23 to a refiner stage 24. The label on the block represent-

ing refiner stage 24 means that it is a refiner, second stage refining, of the less coarse fraction. The refiner stage 24 may comprise a disc refiner conventional in all respects, or it may be a refiner similar to that used in stages 11 and 22 in which a special disc is used in a manner subsequently to be described.

The outputs from refiner stages 22 and 24 are combined and passed through fine screens 25. The rejected wood material from fine screens 25 is returned to drainer stage 21 to become mixed with the coarse fraction from separator 20 and thereby reprocessed through refiner stage 22. The accepted wood material from fine screens 25 goes to a primary centrifugal separator stage 26 to be separated into an acceptable pulp and a primary reject material. The acceptable pulp from stage 26 which may be called a secondary acceptable pulp is combined or mixed with the acceptable pulp from separator stage 16 which may be called a primary acceptable pulp, and the mixed acceptable pulp may then go to a thickening stage 17 or other final stage. The primary reject material from separator 26 goes to a secondary and tertiary separator stage 27 where secondary and tertiary accepted fractions are returned to drainer stage 21 for reprocessing with the coarse fraction from separator stage 20; alternatively the secondary and tertiary accepted fractions may be returned to drainer stage 23 for reprocessing with the less coarse fraction from stage 20. The reject material is discharged as waste, or it may be reclaimed as a by-product.

In the second stages of refining of the wood material, that is in the refining of the wood material not accepted by stages 14 and 16, there are separate refiners for each fraction of this non-acceptable material. Because of this, different degrees and different types of refining can be given to each fraction (coarse and less coarse) as required. The treatment or processing may therefore be adapted to the material being processed and the results required. The overall process is very versatile because of the changes that can be made in it. The amount of energy expended on the wood material by refiner stages 11, 22 and 24 may be varied and the fraction separation by stages 12, 14, 16, 20, 25, 26 and 27 may be varied. The process may readily and conveniently adapted to produce pulps of different qualities for different products. In the case of a coarser final pulp, for example, stages 16, 26 and 27 may be omitted. It will of course be apparent that the non-acceptable wood material from separator stage 16 may be divided into more than two fractions, and each of these fractions may be separately refined as required.

Referring now to FIGURE 2, there is shown a simplified partial side view, mainly in section, of a disc refiner 28 such as may be used in refiner stage 11 of FIGURE 1. The refiner 28 has a casing 30 enclosing a rotating disc 31 and a stationary disc 32. The rotating disc 31 comprises a series of segmented plates 36 bolted or otherwise secured to a backing disc 33 which is supported on shaft 34. The shaft 34 is rotatably driven by a suitable motor (not shown). The rotational speed of the disc should be within the range 900 to 3600 r.p.m. The central part 35 of rotating disc 31 is of a generally conical shape curving outwards towards the inner rim of plates 36. The portion 35 serves as a guide to direct wood chips from the central area outwards between discs 31 and 32.

The plates 36 have a surface that is sinuous in a radial direction. Reference to FIGURE 3 in conjunction with FIGURE 2 will illustrate one form of suitable plates 36. FIGURE 3 shows a plan view of part of two adjacent plates 36a and 36b. Radially extending ribs project from the surface of plates 36 and these ribs are also sinuous or wavelike in a radial direction following the surface of the plates. In other words, the plates 36 themselves and the ribs 47 both have troughs and crests at the same distances from the axis of the disc. The sinuous pattern extends all the way around the disc 31.

The stationary disc 32 also comprises a series of seg-

mented plates designated 37 which are bolted or otherwise secured to a backing member 38. The plates 37 have a sinuous surface provided with ribs, but the plates 37 are designed to mate with plates 36 as shown in FIGURE 2. That is, there is a crest on plates 37 opposite a trough on plates 36. The above waveline plate pattern is of course only one example of a suitable form of plates. Depending on the physical shape of the raw chips and the speed of rotation of the disc other plate patterns and plate orientations may be required for optimum performance. For example, in place of the waveline profile, a sinuous path can still be provided by a first plate pattern similar to the pattern hereinafter recommended for refining stages 22 and 24. For higher speeds, higher pulp consistencies and flatter plate patterns it is desirable to arrange the disc and plates so that there is a tapered gap between the plates 36 and 37 so that the chips leaving the central part 35 will feed into the large end of the taper and progress outward along the sinuous path toward the narrow end of the taper between the plates. This taper may be straight or it may be slightly curved to give a gradually decreasing gap between the plates.

At the higher rotational speeds it may also be desirable to increase the coarser part of the plate area 36b, commonly referred to as the "breaker-bar zone"; here the coarser wood chips are broken up into finer fibrous fragments. For large machines, where the diameter of the rotating disc is for example greater than 45 inches, this can be more easily done without substantially limiting the finer plate area where much of the refining of the fibrous material is carried out.

As hereinbefore mentioned, the rotational speed of the disc should be in the 900 to 3600 r.p.m. range. While superior pulps have been made at the 900 r.p.m. level using moderately high consistencies in the range 6-12%, it has been found necessary to use higher rotational speeds i.e. greater than 1200 when operating at high pulp consistencies in the range 15-25% and higher. These higher speeds help to move the high consistency pulp through the sinuous path it must follow in order to effect the required flexing and fiberizing action. At the lower speeds, the high consistency pulp tends to choke the refiner to the point where the pulp will actually burn. In addition, of course, these higher speeds make it easier, from a purely mechanical and electrical point of view, to supply a high level of power to a given refining unit.

The refiner 28 may have a rotating control ring 40 made up of a plurality of segmented sections 40a, 40b (FIGURE 3), secured to backing disc 33 adjacent the outer periphery of plates 36. While control ring 40 when it is used, may be secured directly to backing disc 33 which is part of rotating disc 31, the control ring is usually considered to be a separate entity and is referred to separately. The control ring 40 may have its surface indented with a series of dimples 48 or may have another pattern incorporated in its surface. A stationary control ring 41, which may be similar to control ring 40 in all respects, is secured to a ring mount 42. Ring mount 42 is adjustably mounted in frame 30 in a known manner for movement towards and away from ring 40. The spacing between facing surfaces of control rings 40 and 41 can thus be adjusted.

Not only is the control ring spacing adjustable, but the entire rotating disc 31 may be moved longitudinally towards and away from stationary disc 32 in a known manner to make the spacing between discs 31 and 32 adjustable. The adjustable spacing of both discs and control rings provides means to adjust the refining process for different pulps properties. The disc spacing is set for a required processing and the control ring spacing adjusted to give a desired rate of movement of wood material radially outwards between the discs. As a result, the length of time the wood material is retained between the discs can be controlled and the amount of energy expended on the wood material regulated.

There are, however, certain types of refiners which are

designed to incorporate other novel features and such a design can make it difficult or impractical for such a refiner to be equipped with a control ring. Under such circumstances where a refiner not equipped with a control ring has to be used, one may, by a careful selection of the various other embodiments of our invention make a pulp with properties similar to the present invention. One such selection, for example, could include proper use of tapered plates in conjunction with higher consistencies and higher rotational speeds.

It will, of course, be apparent that disc 32 in refiner 28 could be a rotating disc also. If both discs were rotating discs they would normally rotate in opposite directions. The refining process of the invention would not be effected by this.

The input to refiner 28 comprises an input guide 43 which conducts wood chips fed into it to a screw conveyor 44 having a screw 45 rotated by a shaft 46. The output from refiner 28 is at the periphery of the discs where material is collected and discharged through discharge outlet 50.

The operation of refiner stage 11 comprising refiner 28 will now be described. Wood chips are deposited in the input guide 43 where they are conducted to screw conveyor 44. The screw 45 of conveyor 44 moves the wood chips towards the central portion 35 of rotating disc 31 where the chips are guided into a path between the rotating disc 31 and the stationary disc 32. While the movement of individual chips may be irregular during the time the chips are between the discs, the over all movement from input to output is a radial movement. As the wood chips move radially outwards along the sinuous path provided between plates 36 and 37 of discs 31 and 32, a mass of chips builds up between the plates. As the chips follow the sinuous path they are subject to continuously recurring flexing action which fiberizes the chips.

It is believed that the improved pulp derived from the first stage refining in refiner 28 may be the result of the great amount of flexing to which the chips are subjected. The flexing produces heat and the combination of the internally produced heat and the flexing action may break the fibre to fibre bonds and so fiberize the chips. The fibre bonds are complex and involve cellulose to lignin bonds and lignin to lignin bonds. It is possible that the heat developed by flexing may raise the temperature of the wood to the lignin softening point.

Thus, while the above describes how a superior mechanical pulp may be produced using a rotational disc speed, plate patterns, plate orientation and pulp consistency all within a certain range, in order to maximize this repeated compression-relaxation action which tends to fatigue the gross woody structure of the material and so release the strong flexible fibrous materials as well as to maximize the wood-to-wood contact, it is desirable to maintain the consistency of the pulp between the plates within the medium to high consistency range (i.e. 5 to 45% based on the oven-dry weight of the pulp). The actual choice of conditions will depend on a number of factors mainly economic in nature. In the case of production units requiring very high production rates, the tendency will be to choose high powered refining units (so as to minimize the number of units) this will require high rotational speeds and this in turn will suggest that the refiners be operated at as high a consistency as is feasible.

In one embodiment of the invention the first stage refiner (refiner stage 11) may be substantially sealed from the atmosphere or pressurized. This will permit more of the heat generated by the flexing action and frictional action to be retained within the refiner, and the refining action will take place in a region of higher temperature. No heat need be applied from an external source to achieve the higher operating temperature which is believed to aid in the breaking of the fibre bonds.

It is desirable in refiner 28 to keep to a minimum the shearing action between the metal surfaces of the plates

and the wood chips. Excessive wood to metal shearing contact abrades and tears the fibres and results in an excessive amount of undesirable chopped up pieces of wood instead of more desirable finer fibre aggregates. To help to keep the metal to wood shearing contact to a minimum and the wood to wood contact and flexing action at a maximum, it is desirable to use discs which have a sinuous or tortuous radial path and also to maintain the spacing between the rotating and stationary discs, or more specifically between plates 36 and 37, greater than about 0.001 inch. The limits of acceptable disc spacing appears to be of the order of between 0.001 and 0.030 inch under most circumstances. The process, however, is very versatile and under some unusual conditions these limits could be exceeded, especially when operating at high consistencies. Normally, when operating in the medium consistency range of 5-15% the spacing will be of the order of between 0.005 and 0.020 inch with a preferred spacing of between 0.005 and 0.010 inch. When using consistencies higher than about 15%, say of the order of 15 to 25% or higher, the plate spacing becomes less critical and a wider range can be used without any ill effects. Generally, the spacing will lie within the wider range 0.020 to 0.100 inches.

As was previously mentioned, in order to increase pulp strength, increased amounts of power can be expended on the wood material in accordance with the process of this invention. To expend more energy in the first stage of refining, that is in the refiner stage 11 of FIGURE 1, the wood must be retained between the discs 31 and 32 (FIGURE 2) for prolonged periods. The passage of wood material radially between discs 31 and 32 may be controlled by changing the plate pattern and/or by changing the control ring spacing. Obviously, if the depth of the waves in the surface of plates 36 and 37 is increased and the slopes of the waves made steeper, the passage of the chips or wood material will be restricted in a radial direction. It is also obvious that the passage will be restricted if the spacing between control rings 40 and 41 is reduced. A restrictive effect may also be obtained by choice of pattern on the control ring. For example, if wood is passing from a coarse sinuous plate pattern to a control ring having a fine flat pattern with a high surface resistance, it will encounter an abrupt change and its flow becomes restricted at the control ring even if the effective spacing between plates and control ring are the same. It is therefore possible to exercise very good control over the energy expended on the chips being processed.

It has been found that an expenditure of energy in the first stage refiner, that is in refiner stage 11 of FIGURE 1, of between about 80 and 200 H.P.D./A.D.T. (horse power days per air dry ton) will give a pulp with a high strength and good drainage properties from the first stage alone. It should be noted that the aforementioned energy values refer to refiner stage 11 alone and not to the overall process. Satisfactory and optimum values for the total process energy for various qualities of pulp are discussed subsequently in connection with FIGURES 5a and 5b.

In the refiner stage 22, the disc refiner may be similar to the disc refiner 28 of refiner stage 11, except it should use the more conventional flatter-type plates having a regular barred pattern. The plate or disc spacing in refiner stage 22 may be much less than that in refiner stage 11 and the wood material is at a medium consistency. In other words, refiner stage 22 may be operated in a conventional manner.

In the refiner stage 24, the disc refiner may be similar to refiner 28 in refiner stage 11, and while it may use conventional-type plates, the preferred plate pattern is that where the surface is indented with a series of dimples. While refiner stages 22 and 24 may be similar to refiner stage 11 and operated in a similar manner the use of higher disc speeds together with the tapered orienta-

tion of the plates permits operation at high consistencies.

While metal plate surfaces have been more generally used for refiner stages 11, 22 and 24, other materials having more abrasive surfaces have been tried (e.g. 5 alundum, carborundum, etc.) and found very effective.

Referring now to FIGURE 4, there is shown a side view, partly in section, of a centrifugal separator or cleaner of the vortex pressure drop type. This type of centrifugal apparatus is known and has been used in the past for removing a small percentage of undesired particles from a pulp suspension. A description of an apparatus of this type and the manner in which it is operated to clean pulp may be found in United States Patent 2,927,693, of Freeman et al., issued March 8, 1960. The apparatus is adapted in the process of this invention to separate a pulp suspension into two major fractions, and it may be conveniently used in separator stage 20. In separator stages 16, 26 and 27, it is used in a more conventional manner.

Briefly, the separator which is designated 49 in FIGURE 4, comprises a barrel portion 51, a cone piece 52, a separation control enclosure 53, and a head piece 54. The head piece 54 has an inlet portion 55 which admits a suspension of wood material and introduces it tangentially into the top of barrel portion 51, at passage 56, to cause a high velocity vortex to occur in the barrel portion 51 travelling down to cone piece 52. Inwardly of passage 56 there is a cylindrical outlet aperture 57 extending upwards to an outlet conduit 58. A first fraction of the 20 wood material passes out the aperture 57 and conduit 58. The first fraction will comprise the lighter particles or fibers which are entrained in the more central upwardly moving portions of the vortex.

The heavier particles are thrown outwardly and settle 35 down the walls into the control enclosure 53. Water or white water is introduced into enclosure 53 tangentially by control inlet 60 to create a vortex. This tends to dilute the downward vortex from cone piece 52 and causes heavier particles or fibres to be thrown against the 40 outer wall of the separation control enclosure 53 and to pass down these outer walls into a collecting ring 61 to discharge through outlet conduit 62. The second fraction comprising heavier pieces of material is thus discharged through conduit 62.

The separation may be controlled as is well known, by 45 varying the amount of water being injected through control inlet 60. As the flow of water is increased through inlet 60 it tends to reverse some of the slower settling particles and entrain them in the inner upward moving vortex, while a decrease in water flow will allow more 50 of the fine fibre to go out the outlet 62. This technique is known as elutriation and the enclosure 53 as the elutriator. Suitable selection of control water flow and of the 55 apparatus dimensions will adapt the apparatus to various consistencies, different wood material input suspensions, and different output fractions. In general, the elutriator is not used for separator stage 20 as the percentage rejection (i.e. the percentage of the second fraction) is very high. Because of its expense and because the use of an elutriator results in dilution of the stock, it is often only 60 used in the last stage of centrifugal separation, such as, for example, in the tertiary separator of stage 27. If an elutriator is not required, then a centrifugal separator not having one is used. This type of separator is well known and is described also in aforementioned United States Patent 2,927,693.

It is believed that the following specific examples of 65 processes in accordance with the invention will aid in providing an understanding of the invention. Reference 70 is made in the examples to the drawings, and in particular to FIGURE 1.

#### Example I

Chip bin 10 was provided with conventional spruce 75 and balsam chips having a moisture content of 45-50%.

The chips were fed into a disc refiner (refiner stage 11 of FIGURE 1) having a sinuous wave-like disc pattern and a dimple control ring pattern as shown in FIGURES 2 and 3. The spacing of the discs or plates was set at about 0.010 inch and the spacing of the control rings about 0.020 inch. While the control ring spacing seems to be such that it would exercise little restricting effect, this is not the case. It should be noted that the disc or plate spacing is measured from the closest points. With the sinuous pattern of the plates used, this spacing would be measured from the tops of the ribs on the facing plates. The plate pattern is fairly coarse and the root of the ribs or the plate surface is considerably different from the top of the ribs. The plate surfaces are therefore, considerably farther apart than the ribs. The control ring spacing, on the other hand, would be measured from the surface of the ring. Consequently, with the spacings used, there is a definite restricting effect exercised on the flow of wood material by the control ring. A contributing factor to this restrictive effect would be the different patterns on the disc and ring as previously mentioned.

The refining consistency in the refiner of refiner stage 11 was about 8%, and the temperature at the input about 50-60° C. with the output temperature about 70-90° C. The energy expended in this stage was about 125 H.P.D./A.D.T.

The output from refiner stage 11 was diluted to a consistency of about 2% and screened using  $\frac{1}{8}$  inch perforated screen plates (coarse screen 12). The reject material from these screens represented about 10% of refiner feed and was returned to the refiner. The accepted portion from coarse screens 12, at a consistency of 1% was transferred to a horizontal centrifugal screen (fine screen 14) equipped with 0.060 inch perforated screen plates. The rejected material was directed to mixing tank 15, while the accepted material, at a consistency of about 0.50% was passed through a centrifugal cleaner of the vortex pressure drop type (centrifugal separator 16). The inlet and outlet pressures respectively of the cleaner or separator were 51 p.s.i. and 1 p.s.i. The accepted pulp from the first stage represented 50% of the total feed.

The non-acceptable wood material was then separated by a centrifugal separator of the vortex pressure drop

5  
10  
15  
20  
25

30  
35  
40  
45

40

45

45

45

45

45

45

45

45

45

45

45

45

45

45

45

45

45

45

45

45

45

45

45

45

45

45

45

45

45

45

45

45

45

45

45

45

45

45

45

proximately zero and the control ring spacing 0.005 inch. The consistency was about 7% and the temperature 50-60° C. About 85 H.P.D./A.D.T. of energy was expended on the less coarse fraction.

The pulps from the second stage refiners (stages 22 and 24) were screened in a horizontal centrifugal screen using 0.060 inch perforated screens (fine screens 25). The rejected wood material was returned for reprocessing in refiner stage 22, and the accepted pulp was then processed through a primary centrifugal separator 26 under conditions similar to those in centrifugal separator stage 16. The accepted pulp from separator stage 26 (secondary acceptable pulp) and the accepted pulp from separator stage 16 (primary acceptable pulp) are blended or combined and represent the total output of acceptable pulp. The primary rejected material from stage 26 was processed through a secondary separator stage and the secondary separator stage rejects were processed through a tertiary separator stage (secondary and tertiary separator stages 27). These separators in stage 27 may also be similar to those in stage 16. The accepted fractions from secondary and tertiary stage separators were returned to refiner stage 22 for reprocessing with the coarse fraction from separator stage 20. The rejected wood material from the tertiary separator in stage 27 was discharged as waste.

In the preceding example, the process conditions were such that the first stage energy expended (refiner stage 11) was 125 H.P.D./A.D.T. Similarly the energy expended in the second stage refiners (stages 22 and 24) was 125 H.P.D./A.D.T. and 85 H.P.D./A.D.T. of the wood material being processed in each of the stages. The energies expended by stages 22 and 24 with respect to the total processed material was approximately 38 and 27 H.P.D./A.D.T., respectively. This gives a total process energy of about  $125+38+27=190$  H.P.D./A.D.T. This is considerably more energy than could be absorbed in a groundwood process for a pulp having the same freeness and it results in a much stronger pulp. For purposes of comparison, various properties of pulp produced by the process conditions in the example, are given in Table I with comparable properties of pulps obtained by two conventional processes.

TABLE I

| Property        | Process of this invention |                   |                   |            | Conventional groundwood | Process of coarse grinding and disc refining |          |            |
|-----------------|---------------------------|-------------------|-------------------|------------|-------------------------|----------------------------------------------|----------|------------|
|                 | Refining stage 11         | Refining stage 22 | Refining stage 24 | Final pulp |                         | Grinding                                     | Refining | Final pulp |
| Energy          | 125                       | 38                | 27                | 100        | 74                      | 42                                           | 28       | 70         |
| Freeness        | 197                       | 51                | 60                | 55         | 90                      | 306                                          | 140      | 125        |
| Bulk            | 2.72                      | 2.39              | 2.45              | 2.36       | 2.5                     | 3.31                                         | 2.54     | 2.49       |
| Burst factor    | 17.1                      | 23.4              | 26.4              | 24         | 15                      | 4.63                                         | 14.5     | 10.2       |
| Tear factor     | 85                        | 60                | 81                | 75         | 45                      | 40                                           | 58       | 42         |
| Breaking length | 3,290                     | 4,330             | 4,475             | 4,000      | 3,200                   | 1,230                                        | 3,130    | 2,350      |
| Fold            | 25                        | 75                | 246               | 201        | 15                      | -----                                        | -----    | -----      |
| Strength factor | 45                        | 45                | 53                | 49         | 30                      | 18                                           | 34       | 24         |

Energy, horse power days per air dry ton; Freeness, Canadian standard freeness; Bulk, cc./gm.; Burst factor, Tappi Standard; Tear factor, Tappi Standard; Breaking length, meters; Fold, double M.I.T. at 0.5 Kg. load; Strength factor, burst  $\frac{1}{2}$  tear.

type into equal fractions each representing about 25% of the total feed. The inlet and outlet pressures of the separator in separator stage 20 were respectively 35 p.s.i. and 1 p.s.i.

After passing through a drainer stage 21, the coarse fraction was processed by a disc refiner (refiner stage 22) equipped with discs having a regular barred plate pattern with a spacing of  $-0.005$  inch and a control ring having a dimple pattern with a spacing of 0.010 inch. The consistency was approximately 7% and the temperature approximately 50° C. The expended energy for the coarse fraction of wood material was about 125 H.P.D./A.D.T. of the coarse fraction.

The less coarse fraction was passed through a drainer stage 23 and was then processed in a disc refiner (refiner stage 24) equipped with discs and a control ring both having a dimple pattern. The disc spacing was ap-

60  
65  
70  
75

Table I indicates that it is possible to expend greater amounts of energy in the process of this invention and thereby increase the strength of the resulting pulp.

#### Example II

Spruce and balsam chips were subjected to a similar process to that of Example I with the following modifications. Refiner stage 11 was provided with a sinuous but flatter barred disc pattern similar to that previously used in refiner stage 22 and the plates were arranged to leave a tapered gap. The spacing of the plates was 0.020 inch at the closest point in the taper.

The consistency in refiner stage 11 was about 25%. The temperature at the input 60° C. and the output temperature about 100° C. The energy expended in stage 11 was about 80 H.P.D./A.D.T. Similarly, the flatter plates, the tapered gap (no control ring) and a consistency of

about 25% was used in refining the coarser fractions in refiner stages 22 and 24. The energy level in these latter stages was approximately 70 H.P.D./A.D.T. giving a total process energy of about 125 H.P.D./A.D.T. While this energy is less than Example I, and consequently the strength of the final pulp was less than that shown in Table I for the previous example, the properties of this pulp were still superior to that for conventional pulps. It will also be appreciated that the use of higher consistencies in the second stages will require more elaborate and expensive thickening equipment than simple drainers (21 and 23) (conventional pulp presses, for example, will serve at these stages). This may be avoided by the use of high consistencies (15% and higher) in stage 11 and lower consistencies (5-15%) in stages 22 and 24.

When a medium pulp consistency is used, as in Example I, the process arrangement allows sufficient time for any tight, localized, high consistency wads or balls of pulp to become disentangled. However, when using high consistencies, as in Example II, such tight balls of pulp are more prevalent and care must be taken to provide the proper conditions for these wads of pulp to become disentangled. While adequate dilution and time are important conditions, higher temperatures and mild agitation will accelerate the opening-up of these fibrous masses.

Referring now to FIGURE 5a, the graph shows strength factor versus total process energy. Curve 64, shown as a solid line, indicates the general relationship between strength and energy input for a pulp made by process in accordance with an embodiment of the invention, while curve 65, shown as a dashed line, indicates the general relationship between strength and energy input for a conventional groundwood pulp. It is apparent from FIGURE 5a that the process of this invention permits increased amounts of energy to be expended on the pulp resulting in improved strength properties. While the total process energy may vary within wide limits, for example between 90 and 300 H.P.D./A.D.T., and achieve improved pulp, better results are achieved when the total process energy is between 120 and 200 H.P.D./A.D.T.

It may be seen that the curve 65 in FIGURE 5a tends to level off with increasing process energy. Consequently, it appears that with a conventional groundwood process, very little increase in strength is achieved by increasing the energy consumption past 80 or 90 H.P.D./A.D.T.

FIGURE 5b in a graph of freeness (Canadian Standard Freeness) versus total process energy. Curve 66, the solid line, indicates a general relationship between freeness and energy input for a pulp in accordance with the invention, while curve 67, the dashed line, indicates the same relationship for a conventional groundwood process. It will be seen that the freeness of groundwood pulp tends to decrease more rapidly than the freeness of the pulp in accordance with this invention for the same increase in process energy.

Referring to FIGURES 5a and 5b together, it will be seen that for a freeness of about 60, the respective energy inputs from curves 67 and 66 would be about 90 and 190 H.P.D./A.D.T. respectively. The corresponding strength factors would be about 31 and 51 respectively. The strength factor for a pulp in accordance with this invention is of the order of 1.6 times that of conventional groundwood pulp. In addition, it appears in practice that the properties of groundwood pulp and pulp produced in accordance with the invention are sufficiently different that identical freeness measurements do not mean identical drainage characteristics of the pulps on a paper machine. The paper machine drainage characteristics of the pulp produced by this invention appear to be better than the freeness measurement (Canadian Standard Freeness) would indicate.

A further embodiment of this invention relates to the pressurization of at least one of the disc refiners used in the process of the invention. Because large amounts of energy are expended in the process, considerable amounts of heat are generated. If a disc refiner, such as refiner 28

of FIGURE 2, were pressurized, steam could be generated within the refiner. This steam would be of the order of 50 p.s.i.g. and could be processed in a reboiler, if necessary, to provide cleaner steam for use in other paper machines. For example, the steam could be used in paper machine driers. In addition the pressurization would enable the refining process to take place at a higher temperature to assist the fiberizing of the wood chips as was previously described.

While the invention primarily relates to a mechanical pulping process, it will be apparent that the advantages of the invention would still be achieved if chemicals were added at some point in the process or if chemically treated or partly cooked chips were used as the starting material. If chemicals are added during the process of the invention, the resulting pulp will be a semi-chemical pulp, but nevertheless the features of the inventive process will be used. Such semi-chemical processes are intended to fall within the scope of the invention. For example, it may be desirable to add a bleaching chemical to the wood material being processed. This may be desirable to brighten the pulp generally, or in the embodiment where steam under pressure is present in one of the refining stages and the refining is at an increased temperature it may be desirable to counteract a possible darkening effect of the pressurized step. If bleaching chemicals are to be added, it is convenient to add them prior to a refining step, for example just before stage 11, so that chemical processing could take place concurrently with mechanical processing.

It will be seen that the present invention provides an improved process for making a mechanical pulp from wood chips.

We claim:

1. A mechanical process for the treatment of raw wood chips using two discs, at least one of which is rotating relative to the other about a common axis, in apparatus having an input at the said axis and an output at the periphery of said discs, comprising the steps of, feeding raw wood chips into said input, directing the movement of the wood chips radially outwards between said discs, causing all the chips to follow a sinuous path as they move radially outwards subjecting the chips to repeated flexing action to fiberize the chips, restricting the discharge at the periphery of said discs to prolong the period of treatment between said discs until between 80 and 200 H.P.D./A.D.T. of energy has been expended on the wood material, retaining heat generated by the flexing action of the chips to generate steam, permitting the pressure created by the steam to rise above atmospheric pressure, and maintaining a desired pressure by withdrawing steam.
2. A mechanical process as defined in claim 1 wherein the relative rotational speed of the discs is in the range 900 to 3600 r.p.m.
3. A mechanical process as defined in claim 1 wherein the refining consistency is in the range 6-12% and the relative rotational speed of the discs is about 900 r.p.m.
4. A mechanical process as defined in claim 1 wherein the refining consistency is in the range 15-25% and the relative rotational speed of the discs is greater than 1200 r.p.m.
5. A mechanical process as defined in claim 2 wherein the refining consistency is in the range 5-15% and the disc spacing is in the range 0.005-0.020 inch.
6. A mechanical process as defined in claim 2 wherein the refining consistency is greater than 15% and the disc spacing is in the range 0.020-0.100 inch.

#### References Cited

#### UNITED STATES PATENTS

- 2,425,024 8/1947 Beveridge et al. ----- 162-236  
2,573,322 10/1951 Ernst ----- 162-236